

## United States Patent Office

2,876,144

Patented Mar. 3, 1959

1

2,876,144

## METAL PICKLING SOLUTIONS AND METHODS

Howard B. Bomberger, East Liverpool, Ohio, and Milton B. Vordahl, Beaver, Pa., assignors, by mesne assignments, to Crucible Steel Company of America, Flemington, N. J., a corporation of New Jersey

No Drawing. Application February 24, 1956  
Serial No. 567,453

9 Claims. (Cl. 134—3)

This invention relates to improvements in pickling solutions and in methods of pickling metals to remove surface scale, oxides and other surface contamination. More particularly, the invention relates to pickling metals like titanium and zirconium and their alloys containing titanium or zirconium as major constituents, which are subject to surface embrittlement due to absorption of oxygen, nitrogen, hydrogen, etc., when heated in air at elevated temperatures such as those required in heat treating or for hot rolling or forging operations or the like. Removal of this embrittled surface layer improves ductility, particularly bend ductility.

Pickling baths or solutions for alloy steels are generally acidic in nature, but most acids commonly employed for the ferrous alloys do not readily attack corrosion resistant metals like titanium, zirconium and their alloys. Among those acids which do, a majority hydrogen-embrittle and/or deeply pit the surface of the metal. Acid pickling solutions which contain appropriate concentrations of fluoride ions constitute important exceptions to the foregoing general observation. Aqueous solutions containing about 10% by weight nitric acid and about 2% hydrofluoric acid have been employed as pickling baths for alloy steels, and these solutions are effective to a limited extent in removing surface scale for titanium, for example. However, they are subject to the following serious limitations: (1) A substantial amount of hydrogen is absorbed by the metal resulting in serious loss of ductility; (2) copious quantities of nitric oxide are produced which react with oxygen of the air to form hazardous nitrogen dioxide in quantities sometimes exceeding available ventilating capacity; and (3) the bath is difficult to control.

In co-pending U. S. patent application Serial Number 435,755, filed June 10, 1954, of which the present application is a continuation-in-part, there is described in detail the basic electro-chemical phenomena which take place during pickling of titanium in such nitric acid-fluoride ion solutions. Therein it is pointed out that there is a critical nitric acid concentration for these fluoride ion-containing pickling solutions, namely, above 15% by weight HNO<sub>3</sub>. When the nitric acid concentration is below 15%, substantial amounts of hydrogen are absorbed by the titanium. The aforementioned application provides an aqueous pickling solution containing from about 15 to 50% nitric acid and about 0.5 to 10% of fluoride ion. At these concentrations the pickling solution gives an acceptable finished surface with a minimum of hydrogen absorption. A solution containing about 30% nitric acid and 4% hydrofluoric acid produced exceedingly good results, dissolving about 0.001" of titanium-7% manganese sheet in a minute at 150° F., with very little hydrogen evolution and absorption by the metal. There

2

is no significant reduction in hydrogen pick-up by the metal at concentrations above 30% HNO<sub>3</sub>, and increase of nitric acid beyond about 50% by weight of the solution is not economical.

5 The only objectionable feature to the nitric acid-fluoride ion pickling solution of the co-pending application is the evolution of poisonous NO<sub>2</sub> gas. This disadvantage may be overcome by the addition to the pickling solution of about 0.5 to 30% hydrogen peroxide. The hydrogen peroxide is itself an excellent oxidizing agent and is more easily reduced than the hydrogen ions formed during pickling. Accordingly, when pickling titanium in a nitric acid solution containing fluoride ions and hydrogen peroxide, the peroxide is reduced to water along with 10 the formation of titanium tetrafluoride, and substantially no hydrogen is evolved which could be absorbed by the metal. Since hydrogen peroxide is itself effective in combination with fluoride ions as a pickling solution, when employed with the nitric acid-fluoride ion solution, the 15 concentration of nitric acid may be reduced. In the co-pending application, an aqueous solution containing from 2 to 50% HNO<sub>3</sub>, 0.5 to 30% H<sub>2</sub>O<sub>2</sub> and 0.5 to 10% fluoride ions was found to be quite effective on the aforementioned metal surface. Solutions of this type give 20 excellent finished surfaces, do not fume, and are the most economical. Optimum results were obtained with such solutions containing about 5% HNO<sub>3</sub>, about 2% H<sub>2</sub>O<sub>2</sub> and about 2% fluoride ions.

Also in the aforementioned application we described 30 a pickling bath for the above metals containing from 0.5 to 5% fluoride ions and from 5 to 35% hydrogen peroxide, i. e., a solution which does not contain nitric acid. This solution has the advantage of no poisonous or otherwise objectional gas evolution; it imparts a good surface finish to the metal treated, and results in very little hydrogen pick-up. The products of the reaction of this 35 solution with the metal treated are simply water and a titanium or other metal complex. Optimum results were obtained with an aqueous bath containing about 20% H<sub>2</sub>O<sub>2</sub> and about 2% fluoride ions. At 150° F. this bath pickled off about 0.001" of metal per minute.

Each of the three types of pickling solutions disclosed in our co-pending application are eminently satisfactory for removing surface scales produced by heat treatment or hot working of titanium, zirconium and their alloys below about 1000° F. However, the aforementioned pickling solutions are not effective for removing scales from metals hot worked or stress-relieved at 1000° F. or higher. Non-uniform pickling occurs, which results 45 in a very rough finish, particularly if the metal surface has been marred by dirt, oil, ink markings, fingerprints, etc., prior to heat treating. Forming and stress-relieving titanium, zirconium and their alloys at temperatures around 1000°—1200° F. is often advantageous in some operations, and accordingly, a pickling solution which will satisfactorily remove the difficult and troublesome films produced on the surface at these temperatures would be highly desirable.

We have discovered that the addition of phosphoric 50 acid to the pickling solutions of U. S. patent application Ser. No. 435,755 produces a pickling bath which is highly effective for removing surface scales from titanium, zirconium and their alloys formed at or above 1000° F. The phosphoric acid modified solutions produce a white, somewhat etched surface instead of the usual lustrous finish. This flat etched finish is often advantageous, especially when a high luster is undesirable, as in finishing

belt-ground sheet, to minimize the appearance of strikes. The present invention contemplates aqueous solutions containing in percentages by weight about 0.5 to 10% of fluoride ions, i. e., hydrofluoric acid or equivalent amounts of fluoride salts, such as NaF, NaBF<sub>4</sub>, NH<sub>4</sub>F, etc., about 0.5 to 10% phosphoric acid, and an oxidizing agent selected from one of the following: about 15 to 50% nitric acid, about 5 to 35% hydrogen peroxide, and about 2 to 40% nitric acid together with about 0.5 to 30% hydrogen peroxide. In most instances, the phosphoric acid concentration will be between 1% and 6% by weight of the solution, with 2% to 5% H<sub>3</sub>PO<sub>4</sub> being preferred. A pickling solution which is particularly effective for removing the difficult light scales formed at 1000°-1100° F. is one containing about 20% HNO<sub>3</sub>, about 3% HF and about 2% H<sub>3</sub>PO<sub>4</sub>. Pickling is carried out in accordance with the present method at temperatures between 100° and 190° F.

A series of tests were conducted to establish that the improved effectiveness of the pickling solutions in removing high temperature scales was definitely attributable to the presence of phosphoric acid, as distinguished from wetting agents often employed in pickling baths, and more particularly, other mineral acids. A sheet of titanium metal was halved and one half scaled in air at 1000° F. for 30 minutes, and the other half scaled at 1100° F. for a like period. Each of the sample sheets was then pickled in a 20% HNO<sub>3</sub>-3% HF bath maintained at 160°-170° F. This solution was used as a standard for comparison. The standard solution did not remove the 1000° F. scale in a satisfactory manner, and gave a rough finished surface. Its action on the 1100° F. scale was considerably less effective, producing a very rough surface. Variations in bath temperature did not have a significant effect upon the ability of the standard solution to remove these oxidized films, nor did any changes in the HF and HNO<sub>3</sub> concentrations of the bath produce beneficial results. The standard solution was then modified by the addition of 0.1% by weight of Quaker State's wetting agent "Queen No. 5." No improvement in pickling was observed on either the 1000° F. or 1100° F. films. Addition to the standard solution of 0.1% by weight of Haas Miller Corporation's surface active agent "Actival 57" likewise did not improve removal of the films. A further series of tests was run with the standard solutions modified by the addition of 5% H<sub>2</sub>SO<sub>4</sub>, 10% H<sub>2</sub>SO<sub>4</sub>, and 5% HCl respectively. There was no apparent improvement in surface characteristics of the sheets pickled in these solutions over those produced by the standard solution.

Phosphoric acid was then added to the standard solution in concentrations of 2%, 5% and 10% H<sub>3</sub>PO<sub>4</sub>. Unexpectedly, the phosphoric acid-containing solutions indicated a definite improvement. Each of the phosphoric acid-containing baths completely removed the 1000° F. scale and entirely satisfactorily attacked the 1100° F. scale on the sample sheets, and in all cases produced a smooth, white, etched surface. Subsequent tests indicated that the addition of only 0.5% H<sub>3</sub>PO<sub>4</sub> to the standard solution produced significant improvements in high temperature scale removal. We observed that for the above standard solution the optimum phosphoric acid concentration appears to be about 2% by weight.

Phosphoric acid additions to H<sub>2</sub>O<sub>2</sub>-HF and

HNO<sub>3</sub>-H<sub>2</sub>O<sub>2</sub>-HF

pickling baths also enable these solutions to satisfactorily remove similar high temperature-produced surface scales. If desired, the improved pickling solutions may be modified by the addition of suitable wetting agents, such as the two mentioned above, which minimize vertical striations produced by nonuniform pickling due to the rapid vertical movement of gas bubbles and solution along the sheet surface.

What is claimed is:

- An aqueous solution for pickling titanium, zirconium and alloys of each with removal of basis metal from the surface without attendant hydrogen embrittlement, comprising in percentages by weight, about: 0.5 to 10% phosphoric acid, 0.5 to 10% of fluoride ions, and at least one member selected from the group consisting of 15 to 50% nitric acid, 5 to 35% hydrogen peroxide, and 2 to 40% nitric acid together with 0.5 to 30% hydrogen peroxide.
- An aqueous solution for pickling titanium, zirconium and alloys of each as set forth in claim 1 comprising in percentages by weight, about 0.5 to 10% of fluoride ions, about 15 to 50% nitric acid and about 0.5 to 10% phosphoric acid.
- An aqueous solution for pickling titanium, zirconium and alloys of each as set forth in claim 1 comprising in percentages by weight about 0.5 to 5% of fluoride ions, about 5 to 35% hydrogen peroxide and about 0.5 to 10% phosphoric acid.
- An aqueous solution for pickling titanium, zirconium and alloys of each as set forth in claim 1 comprising in percentages by weight about 0.5 to 10% of fluoride ions, about 2 to 40% nitric acid, about 0.5 to 30% hydrogen peroxide and about 0.5 to 10% phosphoric acid.
- The method of pickling titanium, zirconium and alloys of each with removal of basis metal from the surface without attendant hydrogen embrittlement, which comprises immersing the metal in an aqueous pickling solution containing in percentages by weight about 0.5 to 10% phosphoric acid, about 0.5 to 10% of fluoride ions, and at least one member of the group consisting of about 15 to 50% nitric acid, about 5 to 35% hydrogen peroxide, and about 2 to 40% nitric acid together with 0.5 to 30% hydrogen peroxide, while maintaining said solution at a temperature of about 100°-190° F.
- The method of pickling titanium, zirconium and alloys of each as set forth in claim 5, which comprises immersing the metal in an aqueous pickling solution containing in percentages by weight about 0.5 to 10% of fluoride ions, about 15 to 50% nitric acid and about 0.5 to 10% phosphoric acid while maintaining said solution at a temperature of about 100°-190° F.
- The method of pickling titanium, zirconium and alloys of each as set forth in claim 5, which comprises immersing the metal in an aqueous pickling solution containing in percentages by weight about 0.5 to 5% of fluoride ions, about 15 to 35% hydrogen peroxide and about 0.5 to 10% phosphoric acid, while maintaining said solution at a temperature of about 100°-190° F.
- The method of pickling titanium, zirconium and alloys of each as set forth in claim 5, which comprises immersing the metal in an aqueous pickling solution containing in percentages by weight about 0.5 to 10% of fluoride ions, about 2 to 40% nitric acid, about 0.5 to 30% hydrogen peroxide and about 0.5 to 10% phosphoric acid, while maintaining said solution at a temperature of about 100°-190° F.
- The method of pickling titanium and its alloys with removal of basis metal from the surface without attendant hydrogen embrittlement, which comprises immersing the metal in an aqueous pickling solution containing in percentages by weight about 1 to 5% of fluoride ions, about 20 to 35% nitric acid and about 1 to 6% phosphoric acid while maintaining said solution at a temperature about 100°-190° F.

References Cited in the file of this patent

UNITED STATES PATENTS

- |           |           |                |
|-----------|-----------|----------------|
| 1,974,570 | Kiefer    | Sept. 25, 1934 |
| 2,564,749 | Bried     | Aug. 21, 1951  |
| 2,598,889 | Caugherty | June 3, 1952   |

## UNITED STATES PATENTS

|           |                |                |
|-----------|----------------|----------------|
| 2,653,085 | Wynne          | Sept. 22, 1953 |
| 2,653,134 | Dilling et al. | Sept. 22, 1953 |
| 2,705,191 | Jumer          | Mar. 29, 1955  |
| 2,705,192 | Laust et al.   | Mar. 29, 1955  |
| 2,711,364 | Beach          | June 21, 1955  |
| 2,711,389 | Beach et al.   | June 21, 1955  |
| 2,736,640 | McGraw         | Feb. 28, 1956  |
| 2,740,700 | Fuller         | Apr. 3, 1956   |

## FOREIGN PATENTS

|        |        |               |
|--------|--------|---------------|
| 75,798 | Norway | Oct. 17, 1949 |
|--------|--------|---------------|

## OTHER REFERENCES

5 Durkin: Metallurgia, vol. 49, page 256, May 1954  
(from October 1953 article).  
Handbook on Titanium Metal, 7th ed., pages 40-44,  
49, 88, 89, 93, pub. by Titanium Metals Corp. of America,  
New York (August 1, 1953).